

A. B. COWDERY,  
PAVEMENT AND PROCESS OF MAKING SAME.  
APPLICATION FILED DEC. 7, 1909.

1,058,848.

Patented Apr. 15, 1913.

2 SHEETS—SHEET 1.

Fig. 1.



Fig. 2.



Witnesses:

M. G. Crozier

Harold S. Lyon.

Inventor,

Arthur B. Cowdery,

by Mitchell, Chadwick & Kent

Attorneys.

A. B. COWDERY.  
PAVEMENT AND PROCESS OF MAKING SAME.  
APPLICATION FILED DEC. 7, 1909.

1,058,848.

Patented Apr. 15, 1913.

2 SHEETS—SHEET 2.

Fig. 3.



Witnesses:

*M. G. Coziers*  
Harold S. Lyon

Inventor,  
Arthur B. Cowdery,  
by *Mitchell, Chadwick & Kent*  
Attorneys.

# UNITED STATES PATENT OFFICE.

ARTHUR B. COWDERY, OF BOSTON, MASSACHUSETTS, ASSIGNOR TO BARRETT MANUFACTURING COMPANY, OF NEW YORK, N. Y., A CORPORATION OF WEST VIRGINIA.

## PAVEMENT AND PROCESS OF MAKING SAME.

1,058,848.

Specification of Letters Patent. Patented Apr. 15, 1913.

Application filed December 7, 1909. Serial No. 531,827.

*To all whom it may concern:*

Be it known that I, ARTHUR B. COWDERY, a citizen of the United States, residing at Boston, in the county of Suffolk and State 5 of Massachusetts, have invented new and useful Improvements in Pavements and Processes of Making the Same, of which the following is a specification.

This invention relates to improvements in 10 pavements and the method of constructing the same.

It is one object of the invention to provide a process for making a firm and durable road at a reduced cost for materials and 15 labor.

It is another object to make a pavement which combines with these qualities of firmness and durability a capability of being repaired effectively by replacement of only a 20 minor portion of its thickness.

To this end the invention provides improved and inexpensive means for sealing the under part of the pavement tight against water and air.

25 It has heretofore been proposed to lay roads in which the foundation consists of broken stones having their voids filled, either with broken stones, or like material, of smaller size, or else with cement or bituminous material. Such filling involves expense, both for the filling material and for the labor 30 of applying it, whether it be worked in with brushes from the top or whether it be mixed with the stones in advance; and in the latter case there is usually additional expense for 35 heating or drying the stones before the mixing occurs, if the material be bituminous; while, if the material be cement it cannot be rolled without being cracked, which entails 40 admission of water and air and leads to an early disruption of the pavement.

By the invention herein described, a substantial part of the labor heretofore involved in making pavement is saved; and also a 45 substantial part of the material with which the voids between the stones have heretofore been filled. At the same time a firm foundation is created and perfectly sealed by a tough and durable upper structure. These 50 objects are accomplished by forming the pavement, except the wearing surface, of

rather coarse broken stone in which the lower portion, for example the lower two-thirds, is rolled firm and is left with its voids unfilled, and the upper portion has its voids filled, preferably with bituminous material, and a zone exists between these two portions which is filled with sand upon which a layer of bituminous material has been placed, which bituminous material works downward somewhat into the sand and upward somewhat about the stones in the upper portion. The voids of the upper portion are filled by grouting the bituminous material into them. The under sides of the stones in 65 this upper portion are bedded in the bituminous material which was placed on the sand and project downward into the top voids of the lower portion, interlocking therewith. The sand forms a bottom for the 70 grouting, preventing it from descending into the voids of the lower portion, so that grouting is needed only to fill the upper portion.

Further features or advantages appear in 75 the detailed description which follows, reference being had to the accompanying drawings in which,

Figure 1 represents a stage in the making of the pavement; Fig. 2 a later stage showing the result of rolling; and Fig. 3 the 80 finished pavement, being a still later stage.

In the drawings the various parts herein-after described are indicated by reference numerals, as follows: The subterrane is marked 10, the first layer of stones 11, the 85 sand 12, the layer of bituminous material thereon 13, the second layer of stones 14; the result of the mixture of layers 12 and 13 by the rolling process is marked 15, the grouting poured from above in the second 90 layer of stones is 16 and the layer of small stones thereon 17 and the top of the wearing surface consisting of bituminous material and sand mixed, 18.

The method or process of making my improved pavement will be understood from a description of one embodiment of the invention, and it will, of course, be understood that the sizes and kinds of material may be varied, and that other variations may be 100 made from the precise method and construction here specifically described, without de-

parting from the scope of the invention or of the patent.

For ordinary purposes the entire pavement may be about six inches thick, substantially all of which is composed of coarse broken stone of uniform grade, as below described.

After excavating to the desired depth, which should in such a case be about six inches below the finished grade desired, the subterrane should be rolled until there are no depressions and then should be filled with about five inches of broken stone of such a size that it has passed through a ring two and one half inches in diameter and has been retained upon a ring one and one quarter inches in diameter; and these stones should then be heavily rolled and compressed until they are firm and present an even surface. On this a layer of sand should be spread loosely, about two cubic yards to each hundred square yards of surface; and, on the sand, liquid bituminous composition, at a temperature of not less than 220° F. should be spread, a suitable amount being about one gallon to the square yard. Over this, more stones of the same size as before are spread, about two and one half inches deep, and are rolled as firmly as possible. Fig. 1 represents the structure before this rolling and Fig. 2 the structure afterward. In this rolling they sink to a thickness of about two inches, and their under sides are driven down through the bituminous composition, and into and through the sand, and into such top voids or openings as exists in the surface of the previously rolled stones, causing, at the same time, some readjustment of said surface stones, by which some of them tip upward and are forced between the stones above them. At the same time the bituminous matter laid upon the sand becomes forced into and mixed with the sand, to a degree, and both it and the sand are forced into whatever openings exist in the top of the mass of stones under them, or are opened therein by the heavy rolling above, until all such entrances to the voids in the structure of stones below are plugged by the sand or by the mixture of sand and bituminous matter. At the same time, the bituminous matter, which, of course, thoroughly coats the bottom sides of the bottom stones deposited upon it, is forced upward on all sides of those bottom stones, thus insuring a perfect bituminous envelop and seal about the under portions of those stones. This coats and makes a firm setting in concrete for the under portions of these stones, which is a result never before attained, so far as I am aware, by any process in which the main portion of the voids immediately under the wearing surface of the road is filled by grouting bituminous material therein, as such material cools so rapidly in contact with

cold stone that it loses its fluidity and does not penetrate the finer crevices nor the larger openings beneath to which they may lead; and of course, it does not at all reach the under sides of the bottom stones.

After the rolling last described, heated bituminous material is to be spread, a quantity of one and one quarter to one and a half gallons to the square yard being approximately suitable, the quantity being sufficient to fill all voids in the upper two inches of stone, in so far as the voids therein have not been filled by the bituminous material and sand rising from below during the rolling. As soon as possible, small sized broken stone should then be spread, between three quarter and half inch size, a quantity of about one cubic yard to a hundred square yards being usually sufficient, and the road should then be firmly rolled and then swept clean of all dirt or particles of stone that may remain unbonded by the bituminous material. Over this may be spread evenly an additional layer of bituminous material, to the amount of about one half gallon per square yard, and covered immediately with sharp coarse sand, after which the road may be rolled again and is ready for use. In the completed pavement there is therefore a wearing surface consisting of bituminous material and sand and small stones which seals the pavement at the very top and is bonded to the six inches or so of coarse stones and is, to a degree, embedded in the top voids thereof. The upper third of this six inches is of strong and sizable stones in which the voids are completely filled with bituminous material and the under sides of the stones enveloped and firmly bedded in bituminous material. This two-inch layer is mechanically locked with the firm structure of similar stones beneath by the downward projecting points of its lower stones and the upward projecting points of the upper stones of the said under portion. The zone of sand, intervening where these two portions adjoin, served the function, during construction, of holding the bituminous liquid upon the surface until the upper stones were spread in it, thus coating the under sides thereof completely, and of holding the bituminous material further while it and the sand and the adjacent portions of stones above and below the sand were intermingled and kneaded, by the rolling, into a firm stable mass of concrete, supported on a structure of coarse stones with empty voids between them. This upper two inches as thus described, with the dam of sand and concrete under it is relied upon to exclude air and water from the voids below. As a preliminary matter, the foundation should be subdrained if necessary, to keep water from running into it from the sides.

In a foundation thus constructed, the

voids of the lower portion remaining unfilled, the cost of materials to fill them is saved; and the cost of filling them, whether by preliminary mixing or by rubbing the 5 filler in from the top, is saved. The rolling of the stones will naturally be such as to close the voids as much as possible, without rounding the stone, and if this be done the stones will lie in firm jointure, and will 10 be as a mass, in stable equilibrium.

The top portion constitutes a perfect concrete and differs from other concrete in that it is formed and kneaded *in situ*, without preliminary mixing or heating of stones, 15 and by the very simple processes of spreading, of pouring, and of rolling. This is further considerable saving in labor. By the use of bituminous or asphaltic binder by this method it is possible to leave unfilled 20 the voids of the greater part of the six inches thickness of pavement, because such a binder is so elastic that it will endure the greater degree of concussion and of variations of temperature and pressure which a superficial layer receives, as compared with a 25 solid layer from top to bottom; so that the filling from top to bottom which has hitherto been necessary where cement has been used is obviated.

In the same manner the pavement whose 30 construction has been described allows for repairs of the top of the road upon removal of about two inches. A patch can then be put on and will adhere to the existing 35 foundation without necessity of removing the material to the very bottom in order to get firm adhesion.

If it be desired to apply the invention to the improvement of an existing road, the 40 said existing road may in many cases be utilized as the lower element in the improved road, in place of the bottom layer of broken stones with empty voids, as above described, in which the individual stones 45 lie in whatever relation to each other they are thrown by chance. In such cases the top of the existing road, which may be any kind of a road capable of furnishing a firm support for the sand and upper body, 50 should first be washed or swept out to remove all dirt and then the above described successive layers of sand, bituminous binder, coarse stone, grouting, and wearing surface may be applied. In some cases, particularly 55 where the existing road has an asphaltic surface or other sort of fairly smooth surface without top voids, it may be well to first coat such surface with some suitable material which will stick to it and to which 60 the layer of sand will stick. When the bituminous binder has been applied above the sand and the stones, and all rolled, the resulting concrete mass will then adhere to the former existing road sufficiently to prevent 65 lateral displacement.

It will be understood that the fine material for the wearing surface at the very top is put on to make a suitably smooth finish, as has long been practiced in road making, and that this may be of any suitable construction, or may, if desired, be omitted altogether without affecting the essential features of the invention. For these reasons mention of the finer materials added to finish the top of the pavement is omitted in 70 the claims.

I claim:

1. The method of constructing a pavement which comprises spreading a layer of coarse broken stone; rolling till firm; 80 spreading sand or the like loosely on it; spreading thereon liquid bituminous binder; spreading upon that more broken stones; driving the latter stones down into interlocking relation with the first mentioned stones by rolling the whole; and grouting with liquid bituminous binder to fill the voids in the last applied stone.

2. The method of constructing a pavement which comprises providing a firm under support; spreading sand or the like loosely thereon; spreading liquid bituminous binder on the sand; spreading coarse broken stones over said liquid; mixing the sand and binder into concrete and surrounding the 90 under portions of said stones with such concrete by rolling said stones; and applying a liquid grouting to fill the voids in said stones.

3. A pavement comprising a body of stone broken coarsely in irregular shapes, the 100 position of individuals in said body of stone being arranged by chance with projecting corners intervening between other stones in the body whereby a structure of interlocked individuals of approximately the same size is constituted; and said body having intermediate of its height a layer of sand and bituminous binder mixed; the voids in the 105 stones below the said sand layer being empty; and the stones above said sand layer being surrounded and their voids filled with bituminous binder supported on the sand.

4. A pavement formed in layers comprising coarse broken stone at the bottom with the voids therein empty; sand resting on said stone and filling the top voids thereof; bituminous binder supported on the sand; coarse broken stone thereon, having its under sides coated and its voids filled with bituminous binder supported by the sand layer; said coarse stones being broken in irregular shapes of approximately the same size and the individuals in the two layers interlocking with each other through the said intervening bituminous binder and sand.

5. A pavement formed in layers comprising a firm under-support having an irregular upper surface adapted to receive and 110

interlock with stones above it; a layer of sand supported thereon; bituminous binder retained by the sand; coarse stones broken into irregular individual shapes having projecting corners penetrating the binder and sand and interlocking with said support, these stones having their under sides coated and their voids filled with bituminous

binder retained in position by said sand layer. 10

Signed by me at Boston, Mass., this 6th day of December, 1909.

ARTHUR B. COWDERY.

Witnesses:

JOSEPH T. BRENNAN,  
EVERETT E. KENT.